

Sept. 2, 1952

A. H. RISHOI ET AL

2,608,759

DEVICE FOR HANDLING BUTTER AND LIKE MATERIALS

Filed May 13, 1943

2 SHEETS—SHEET 1



Inventors:  
Alfred H. Rishoi,  
Charles F. Weinreich,  
Lorrus Burrell,

By Norman E. H. Heiletzke  
Atty.

Sept. 2, 1952

A. H. RISHOI ET AL

2,608,759

DEVICE FOR HANDLING BUTTER AND LIKE MATERIALS

Filed May 13, 1943

2 SHEETS—SHEET 2

Fig. 3.



Fig. 4



Fig. 5.



Fig. 6.



Fig. 7



Fig. 8.



Inventors:

Alfred H. Rishoi,  
Charles F. Weinreich,  
Loorus Burrell.

By Norman E. H. Fleetzke  
Atty.

## UNITED STATES PATENT OFFICE

2,608,759

## DEVICE FOR HANDLING BUTTER AND LIKE MATERIALS

Alfred H. Rishoi, Wilmette, and Charles F. Weinreich, Des Plaines, Ill., and Loomis Burrell, Little Falls, N. Y., assignors to Cherry-Burrell Corporation, Wilmington, Del., a corporation

Application May 13, 1943, Serial No. 486,816

5 Claims. (Cl. 31—33)

1

This invention relates to new and useful improvements in devices and the like for handling oleaginous materials, such as butter and fats, which normally have a tendency to adhere to surfaces with which they come in contact. More particularly this invention relates to improvements in surfaces for contacting materials. The improved surfaces are adapted to receive a film of liquid, such as water, and are capable of retaining such a film of liquid while being subjected to friction and percussive impact in the handling of fatty or oily materials.

This invention is particularly well adapted for use in churns and butterworkers and in other similar devices, such as butter molds and printers. The invention will accordingly be described in its preferred embodiment in a churn and butterworker. The invention is, however, equally well adapted for use in other devices for the handling of other products which have the characteristics of tending to adhere to dry surfaces of handling devices in a similar manner as is commonly experienced in the handling of butter.

The aspect of the applicants' invention which pertains to "A Method of Churning and Working Butter" is disclosed and claimed in the applicants' co-pending divisional application Serial No. 88,014, filed April 16, 1949.

In conventional churns and butterworkers, particularly commercial varieties, the butter-contacting surfaces are commonly constructed of wood. In some isolated instances the butter contacting surfaces consist of enameled or glazed surfaces which have been etched or sandblasted. In still other instances the butter contacting surfaces of such devices have been made of etched or sandblasted metal sheets. In some instances the butter contacting surfaces in butter handling devices have been made of cast metal or a combination of cast metal and wood.

The use of wood in the construction of churns and butterworkers has been commonplace for many years. The wood construction has the advantage that the butter during the churning and working operation does not normally adhere to the moistened wood. This is probably due to the fact that the porous wood which possesses good wetting and water absorbing and retaining properties, after first having been moistened, is capable of and does retain a film of liquid which prevents the direct contact between the surface of the wood and the surface of the butter within the churn, thereby preventing the objectionable adhesion of the butter to the wood. Obviously such a film of liquid must be capable of with-

2

standing the friction and impact of a mass of butter as it is being worked within the churn. Due to the fact that wood is capable of absorbing a substantial quantity of moisture it is also capable of replenishing the moisture within the film on the surface of the wood as that film may from time to time in certain instances be absorbed by the butter due to the frictional or percussive engagement with the butter.

There are, however, various objections to the use of wood or like materials in the construction of receptacles or other devices for handling a material, such as butter, and particularly for the handling of food products which must be maintained in a clean and sanitary condition. A wooden churn drum, especially when new, may impart an objectionable woody flavor to the butter. The porosity of the wood and the seams between adjacent wooden members embodied in a churn drum, by virtue of which porosity and seams the wooden churn drum is capable of absorbing and holding quantities of water, which enables the very satisfactory retention of a film of water on the surface of the wooden members, is also the reason why a wooden churn drum is difficult to clean and sterilize.

Obviously when the wooden members of the churn drum absorb water they may also absorb food matter which may lodge in the sub-surface of the wood, thereby impeding sterilization and cleansing of the churn drum and enhancing the likelihood of contamination of the churn ultimate contamination of the butter. It is common knowledge that churns constructed of wood, if not meticulously cleaned and sterilized, which cleaning and sterilizing is extremely difficult, lend themselves well to the development of molds and yeast which tend to contaminate the churns and ultimately contaminate the butter. The tendency of wood to warp, shrink and decay is an additionally objectionable feature of the use of wood for the construction of churn drums. These objectionable characteristics of wood present structural and sanitary problems in the design, construction and use of churn drums made of wood.

One of the chief objections to the use of glazed, enameled or glass-lined surfaces in a churn and butterworker is the ever present danger of chipping of the enamel or glass surfaces and the resultant danger of incorporating such foreign matter in the ultimate butter product. It has also been found that etched or sandblasted surfaces of glazed, enameled or glass-lined churns do not satisfactorily retain a film of liquid to prevent the

adhesion of butter thereto. The use of sandblasted metal surfaces, though satisfactory from a sanitary standpoint and though lending themselves well in the construction of a churn and butterworker, is, however, objectionable for the reason that the sandblasted sheet metal surfaces do not appear to possess the qualities necessary to retain a sufficiently strong film of liquid essential to withstand the friction and percussive impact experienced in the normal butter churning and working operations.

Cast metal in certain instances does appear to be capable of retaining a suitable film of liquid to permit the satisfactory use thereof in the construction of churning and butterworkers. However, the construction of large cast metal churning adapted for use as commercial churning and butterworkers is difficult and costly and requires the use of objectionably large quantities of metal in the large, heavy castings.

It has been found in this invention that sheet material, such as sheet metal, when properly prepared as, for example, by sandblasting, metalblasting or suitable machining, to thereby impart a rough surface to the sheet metal, to which roughened surface is added an auxiliary porous surface coating as, for example, by metallizing or the like in the instance of the use of sheet metal, will satisfactorily retain a film of liquid of sufficient strength to withstand the friction and percussive impact of large quantities of butter or the like as they are being churned and worked in a large commercial churn provided with the improved material contacting surfaces.

In the preferred embodiment of the invention there has been provided a metallized surface imposed upon a sandblasted or otherwise suitably roughened surface of a sheet of rolled or worked metal, preferably stainless steel. The selected metal, in the instance of the metallizing substance and the rolled or worked sheet metal, may, of course, be of various types. In each instance it is, however, desirable to select metals from the group commonly referred to as stainless metals for the reason that these metals are substantially non-corrosive and do not readily react with the ingredients normally found in a dairy product, such as butter.

In the selection of metals for use in the construction of churning and butterworkers embodying the instant invention, the factors of availability, durability, resistance to corrosion, chemical reaction with the product handled, wetting properties, liquid absorption and liquid film retaining and replenishing capacity, and cleaning and sterilizing properties should be considered. Numerous combinations of metals and types of treatment of the metals have been experimented with and it has been found that such sheet metals as tinned iron, aluminum, and ordinary irons and steels are all generally objectionable for the reason that they are usually subject to excessive corrosion and in some cases enter into an objectionable chemical reaction with such products as milk and butter.

Obviously any metal or group of metals selected must also lend itself well to fabrication of the desired type of receptacle or material handling device. Comparative tests were made on wood, cast aluminum, metalblasted and sandblasted aluminum, metalblasted and sandblasted sheets of stainless steel metallized with aluminum or stainless steel or other steel alloy, sandblasted glass, chemically corroded stainless steel, heat treated stainless steel in which intergranular cor-

rosion has been induced by heat treatments to cause precipitation of chromium carbide, and sheet tin, iron, steel and copper treated in the various combinations of sandblasting, metalblasting and metallizing.

During the comparative tests of various combinations of metals and alloys as above referred to and other materials, such as glass and enamelware, it was found that the fine-grained butter contacting surface was not as desirable as a relatively coarse-grained surface. It was also observed, with respect to certain metals, that the metallizing process apparently decreased the resistance to corrosion of the normally non-corrosive base or supporting metals. It was found that coarse-grained, preferably sandblasted, stainless steel sheet metal of the 18-8 variety metallized with Inconel, a trade-mark of the International Nickel Company used to identify an alloy containing approximately 13 per cent chromium, 6½ per cent iron, and 79½ per cent nickel, possessed the desirable characteristics of durability, satisfactory resistance to corrosion, good wetting properties, and good liquid absorption and liquid film retaining and replenishing properties. The alloy 18-8 is an improved corrosion resistant alloy, as described in various authoritative publications, such as the "Metals Handbook of the American Society for Metals" (1939 edition), page 541; the Monograph of the American Chemical Society, monograph series, entitled "Corrosion Resistance of Metals and Alloys," by Robert J. McKay and Robert Worthington, published by the Reinhold Publishing Corp., 330 West 42nd Street, New York, N. Y., 1936; and the Bulletin T-7 (revised as of January 1939), "Property and Uses of Inconel," published by the Development and Research Division of The International Nickel Company, Inc., 67 Wall Street, New York, N. Y. It was also found that such a roughened, stainless steel surface metallized to the desired extent with Inconel was also readily cleaned and sterilized.

It should be noted that satisfactory results were also obtained when the stainless steel surface was roughened by metalblasting instead of sandblasting. It was discovered that the slight tendency of the metallized surfaces of the stainless steel to corrode was substantially reduced when the metallizing process was performed in an atmosphere of inert gas to prevent the oxidation of small particles of molten or semi-molten metal as they were percussively impacted against the roughened surface of the base metal to which they adhere primarily by a mechanical bond. Suitable base surfaces for metallizing may also be produced by appropriate machining operations.

It is, of course, common knowledge that the chemical composition of butter, particularly salted butter (sodium chloride), is such as to tend to corrode many of the common metals and alloys which otherwise may be satisfactory for use in the embodiments of the present invention. The selected metals, alloys or other compositions, such as plastics, for use in the present invention must be such as will not be readily affected by the chemicals present in a product, such as butter, to be handled.

The prime object of the present invention is to provide a surface for contacting butter and like materials in which the surface is adapted to receive and retain a film of liquid; in which the surface is of such a structure as may be readily cleaned and sterilized; in which the surface material lends itself to the ready fabrication

of receptacles, such as drums for churns and butterworkers, and other similar devices, such as molds and printers; in which the surface is durable and may be produced from readily available materials; in which the surface is appreciably resistant to corrosion and substantially neutral in its effect on butter; in which the surface possesses the characteristics, when moistened, of preventing the ready adhesion thereto of a substance, such as butter; and in which the surface possesses the quality, when moistened, of absorbing or retaining a reserve supply of liquid to replenish the surface film.

The foregoing and other objectives and advantages of this invention will become more apparent during the course of the following description when read in connection with the accompanying drawings in which:

Figure 1 is an illustrative elevational view, partially in broken-away section, of a churn and butterworker embodying the improved surface of the present invention.

Figure 2 is a vertical sectional view taken along line 2—2 of Figure 1.

Figure 3 is a reproduction of a photomicrograph showing on a greatly enlarged scale in portion A thereof the surface characteristics of a metalblasted, stainless steel, sheet metal surface contrasted with portion B thereof in which the metalblasted surface has been metallized with Inconel.

Figure 4 is a reproduction of a photomicrograph showing on a greatly enlarged scale the surface characteristics of a stainless steel, sheet metal surface sandblasted with coarse sand grit.

Figure 5 is a reproduction of a photomicrograph showing on a greatly enlarged scale the surface characteristics of a metalblasted surface of sheet aluminum upon which aluminum has been metallized.

Figure 6 is an illustrative sketch depicting in a grossly exaggerated manner a cross section of a sheet of metal which has been sandblasted or metalblasted to produce an irregular surface thereon and then metallized, the illustrated metallized portions of metal being generally identified by the letter D, together with a film of liquid identified by the letter E.

Figure 7 is a reproduction of a photomicrograph showing on a greatly enlarged scale the surface characteristics of sandblasted stainless steel sheet metal metallized with Inconel.

Figure 8 is a reproduction of a photomicrograph showing on a greatly enlarged scale the surface characteristics of a metalblasted sheet of stainless steel sheet metal.

Referring now to the drawings, in which like numerals identify like elements, the reference character 10 identifies churn supporting elements, one of which houses a power unit for rotating the churn drum 11. The churn drum 11 is supported by rotatable gudgeons 12 pivoted on the frame elements 10. The drum 11 consists of a horizontally disposed cylindrical outer shell 13 preferably made of sheet metal and provided with opposed drum heads 14 of like material.

The drum heads 14 are sealed to the ends of the cylinder 13 and affixed thereto in any conventional manner, such as by welding. The gudgeons 12 are secured to the drum heads 14 in any conventional manner, such as by welding.

An inner cylindrical sheet metal liner 15 is similarly provided with drum heads 16 and is housed within the outer shell 13 and supported

in spaced relation to said shell 13 and outer drum heads 14 by spacing elements 17. Alined openings are provided in the walls of the concentric cylinders 13 and 15, which openings are sealed by a sheet metal door 18.

Within the inner cylinder and rigidly fixed thereto there are provided a tubular, preferably sheet metal, element 19 and butter churning and working shelves 20 also made of sheet metal. The cylinders 13 and 15 are sealed one to the other in any conventional manner about the alined openings sealed by the door 18. The surfaces of the element 19, shelves 20, inner churn liner 15 and inner drum heads 16 are all provided with the improved butter contacting surface which, in the preferred embodiment, consists of sandblasted stainless or rust resistant steel of the 18-8 variety, which sandblasted surface has been suitably metallized with Inconel or similar metal containing at least 18 percent chromium. The improved surfaces in Figures 1 and 2 are generally indicated by the letter C and are illustrated on a greatly enlarged scale in Figure 7.

The process of sandblasting or metalblasting and metallizing utilized in the preparation of the preferred butter contacting surface as just described is well known in the sandblasting, metalblasting and metallizing arts and no improvement in the art of sandblasting, metalblasting or metallizing constitutes a part of the invention claimed herein. The present invention consists in the discovery that suitably metallized or similarly treated surfaces C as afore-described possess the capability of receiving, maintaining and, when necessary, replenishing a tenacious film of liquid B, upon being moistened, which film adapts them for use in devices for the handling of substances, such as butter and the like, which substances normally tend to adhere to similar surfaces when dry, but do not tend to adhere to the improved surfaces when moist due to the film of liquid thereon.

Particular combinations of metals and alloys have been selected for the preferred embodiment of this invention in view of their availability, resistance to abrasion, resistance to corrosion, neutral reaction with butter and the like, and their ability to receive, maintain and replenish a film of liquid under adverse conditions of friction and percussive impact with the material or substances handled, such as butter and other fatty materials. It has also been found that aluminum or aluminum alloy sheet metal, when properly roughened and metallized, though not as durable as the selected combination of stainless steel and Inconel, is, however, capable of receiving, retaining and replenishing a strong film of liquid.

In the preparation of the surface of the preferred embodiment of the invention, a sheet of stainless or rust resistant steel metal, containing at least 18 percent chromium, of the 18-8 variety is first sandblasted. During the sandblasting process, grit, such as any suitable sand well adapted for blasting metal, of varying coarseness may be used so as to produce the desired varying degrees of roughness of the sandblasted sheet. If desired, the base sheet of stainless steel metal may also be roughened by metalblasting the same with metal particles of the desired coarseness.

After the base sheet of stainless steel metal has been properly roughened by either the metalblasting or sandblasting process, or by a suit-

able machining process, and after all foreign material has been removed therefrom and while it is clean, the metallizing coating should be applied in such a manner as to secure the desired degree of interlocking between the roughened surface and metallized particles and to the desired degree of roughness and porosity or spacing of the metal particles one from another and between portions of the metal particles and the face of the metallized surface. The metallizing process should preferably be carried out in an atmosphere of inert gas which tends to inhibit corrosion of the resulting surface.

Though the invention has been described with reference primarily to a metallized sheet metal surface, it is, of course, to be understood that a similar type of surface produced by the application of minute particles of plastic substances upon a suitably roughened base of plastic material is also contemplated by this invention.

In the operation of a churn and butterworker embodying the improved surface of this invention, after the surface has been moistened with liquid, such as water, to form a film thereon, the desired quantity of cream of the consistency and at the temperature preferred is introduced into the churn drum. The churn is then rotated at a suitable speed until the desired agglomeration of the butter fat globules in the cream is effected after which the buttermilk is drained from the churn drum. Water may then be added to the agglomerated mass of butter flakes and the mass washed by rotating the churn drum, after which the water or other washing liquid is also drained from the churn. The churn is then further rotated at a satisfactory speed for a suitable period of time to work the butter and, if desired, predetermined quantities of salt and water may be added for uniform distribution throughout the mass of butter. As will be apparent upon an inspection of Figures 1 and 2 of the drawings, the mass of cream and also the mass of butter, during the phases of the various churning and butterworking operations, will be percussively impacted against the improved surfaces of portions of the interior of the churn drum, shelves and central element. Obviously during the rotation of the churn drum, the mass of butter, as it is being worked, will also slide over the moistened surface of the exposed elements of the interior of the churn drum, shelves and central element.

It will be apparent that by this invention there has been provided an improved surface readily adaptable for use in devices, such as churning and butterworking, molds, printers, etc., which surface may be made from readily available materials and possesses the desired qualities of durability and resistance to corrosion.

The improved surface and associated materials lend themselves readily to fabrication, cleaning and sterilizing and are substantially neutral in their effect on butter and like products. Due to the ability of the improved surface to retain within its artificially produced pores a suitable quantity of liquid, when moistened, and to retain and maintain a tenacious surface film of liquid, when moistened, the improved surface is particularly well adapted for use in devices used in the handling of butter and like fatty materials, which materials would otherwise tend to adhere to the surfaces of the devices.

Although the invention has been primarily described with respect to the preferred embodiment thereof incorporated in a churn and butterworker and constructed of the preferred metals and

alloys, various modifications of the improved butter and the like contacting surfaces within the scope of the invention will be apparent to those skilled in the art upon a review of the foregoing description and the appended claims.

The invention is hereby claimed as follows:

1. A device for use as a churn and butterworker comprising a sheet metal drum provided with a roughened inner surface, said drum being formed from a rust-resistant alloy containing at least 18 per cent chromium and a covering layer of an alloy containing at least 18 per cent chromium which has been applied to said roughened surface by metallization, whereby a butter contacting surface is secured, which surface when moistened will not readily adhere to butter.

2. A device for the handling of butter-like products comprising a sheet metal drum provided with a roughened inner surface, said drum being formed of rust-resistant aluminum and metallized with a covering inner layer of aluminum, whereby a contacting surface is secured, which contacting surface when moistened will not readily adhere to butter-like products.

3. A device for the handling of butter-like products comprising a sheet metal drum provided with a roughened inner surface, said drum being formed of a rust-resistant alloy and metallized with a covering inner layer of aluminum alloy, whereby a contacting surface is secured which contacting surface when moistened will not readily adhere to butter-like products.

4. A device for the handling of butter-like products comprising a sheet metal drum provided with a roughened inner surface, said drum being formed of rust-resistant aluminum and metallized with a covering inner layer of minute particles of aluminum secured to said surface, whereby a contacting surface is secured which contacting surface when moistened will not readily adhere to butter-like products.

5. A device for the handling of butter-like products comprising a sheet metal drum provided with a roughened inner surface, said drum being formed of a rust-resistant alloy and metallized with a covering inner layer of minute particles of a rust-resistant alloy secured to said surface, whereby a contacting surface is secured, which contacting surface when moistened will not readily adhere to butter-like products.

ALFRED H. RISHOI,  
CHARLES F. WEINREICH,  
LOOMIS BURRELL.

#### REFERENCES CITED

The following references are of record in the file of this patent:

#### UNITED STATES PATENTS

| Number       | Name           | Date           |
|--------------|----------------|----------------|
| 681,068      | Noack          | Aug. 20, 1901  |
| 1,002,431    | Noack          | Sept. 5, 1911  |
| 1,540,761    | Chormann       | June 9, 1925   |
| 65 1,885,626 | Quaedvlieg     | Nov. 1, 1932   |
| 1,973,740    | Andres         | Sept. 18, 1934 |
| 2,108,162    | Clark          | Feb. 15, 1938  |
| 2,200,513    | Mitchel et al. | May 14, 1940   |
| 2,200,514    | Mitchel et al. | May 14, 1940   |
| 70 2,320,327 | Meduna         | May 25, 1943   |

#### OTHER REFERENCES

"Handbook of Chemistry and Physics," twenty-third edition, published in 1939 by Chemical Rubber Publishing Co., Cleveland, Ohio, page 888.